

April 18, 1967

F. S. TOBEY

3,314,816

METHOD OF MAKING PHOTOGRAPHICALLY ACCURATE PRINTS

Filed Aug. 2, 1962



3,314,816  
METHOD OF MAKING PHOTOGRAPHICALLY  
ACCURATE PRINTS

Frederic S. Tobey, Walpole, Mass., assignor to W. H. Brady Company, Milwaukee, Wis., a corporation of Wisconsin

Filed Aug. 2, 1962, Ser. No. 214,282  
1 Claim. (Cl. 117—101)

This invention relates to a method for making prints with photographic accuracy and without any layer of gelatin or the like.

Photographic prints heretofore familiar to the art have typically included a layer of soluble organic material, such as gelatin, and, arranged therein to define photographic images, particles of silver. Such prints have various disadvantages.

One disadvantage, for example, is that at higher temperatures such organic materials decompose and produce discoloration destroying in effect the photographic images, so as to make impractical use of such prints as indicia-bearing labels for many applications, despite the desirability of such use, particularly where indicia of small size and high resolution (for reading by means of a magnifying glass, in connection with miniaturized components, for example) are needed.

I have discovered a method of producing prints with photographic accuracy and precision which makes possible elimination of layers of organic material (such as the hydrophilic colloids gelatin, albumen, hydrolyzed cellulose esters, and hydrolyzed polyvinyl acetates) carrying dispersed therein image-defining solid particles, and provides prints characterized by high temperature stability, increased moisture stability, and great flexibility. Further advantages of my new method are that a positive print may be made directly from a conventional positive photographic print or transparency, or a negative print may be made directly from a conventional negative photographic print or transparency; and if desired a print may be produced in which the solid particles extend, arranged still with photographic accuracy, well below the surface thereof, providing the additional advantage that if the surface becomes illegible, as because dirty, it may be buffed off to reproduce a legible image.

Generally speaking, in my new method I take a base on which I wish to produce a print and I also take a layer of organic material in which are dispersed solid particles of material defining an image which the finished print should carry. I then dispose the layer of organic material and the base (which may or may not be integral with each other) away from an axis of rotation, with the base further from the axis than the layer and the layer between the axis and the base, support the layer and base in this relationship, and rotate the layer and base while so supported simultaneously and with the same angular velocity about said axis. While maintaining this condition, which biases the organic layer and the image-defining solid particles carried thereby radially from the axis toward the base, I introduce a solvent which is specific to the organic layer, to dissolve the same without dissolving the image-defining solid particles or the base. The solvent destroys the integrity of the organic layer, whereupon the solid particles move along radial paths away from the axis and impinge on the base, to produce a print in which said solid particles are carried in image-defining relationship by said base.

If desired, said base or the receiving surface thereof may be made so porous that the solid particles are driven well below the surface thereof.

The base may comprise any suitable material, including for example blotting or bond paper, glass cloth, or a plastic, for example Mylar. The organic layer may be

dissolved using any suitable solvent which will destroy the integrity thereof without similarly affecting the solid particles or the base; when the organic material is gelatin, for example, it may for example be dissolved in water solutions of sodium hydroxide or papaya extract; suitable commercial preparations familiar to the art in processes to reclaim silver from prints and transparencies are Gelatinase No. 3, manufactured by Miles Chemical Co., Clifton, N.J., and S.P.C. Enzyme Photo-Film Remover, manufactured by Wallerstein Co., Staten Island, N.Y. The organic layer may if desired be given a preliminary softening treatment with such a solvent prior to destroying the integrity of the organic layer by solvent action.

There is shown in FIG. 1 an apparatus in which the process is being practiced, starting with a conventional positive photographic print. FIG. 2 is an enlarged sectional view at an early stage in the practice thus of the process, taken at 2—2 of FIG. 1. FIG. 3 is a view corresponding to FIG. 2, but at a later stage of this embodiment of the invention. Thicknesses of silver and organic material have been shown disproportionately, in the interest of clarity.

Electric motor 10 rotates drive shaft 12 which in turn rotates perforated basket 14 about the axis of said shaft. Solvent or wash liquid may be introduced as desired through pipe 16, and removed through pipe 18. The process is shown in the drawings as applied to a conventional photographic print, in which silver particles 20 are disposed to define photographic image in a gelatin layer 22 which is adherently integral with a layer of paper 24. As will be seen, in FIG. 3 the gelatin originally present as shown in FIG. 2 has been removed, and the silver particles 20 have migrated along radial paths without disturbing the image onto and into interstices of the paper support 24 (dimensions of course being greatly distorted in the figures for clarity).

Preferred embodiments of the new method and product of the invention will now be set forth. In all the following examples good adhesion and good resistance to distortion from rubbing resulted.

*Example 1*

The gelatin layer of a conventional photographic print (in which a developed and fixed photographic emulsion, constituting particles of silver carried in photographic arrangement in a layer of hardened gelatin, was integral with a carrier layer of good quality paper) was first softened without destruction of its integrity by soaking the print for ten minutes at room temperature in a dilute solution of sodium hydroxide. The print was then placed in a centrifuge basket against an imperforate cylindrical wall thereof, and liquids were added on a batch basis. The gelatin-silver layer was placed radially inwardly, and the print was rotated about the axis of the cylindrical centrifuge basket (which was ten inches in diameter) for ten minutes at 5,000 times gravity in the presence of the same dilute sodium hydroxide solution. Rotation was repeated for ten more minutes under the same conditions, except that water was substituted for sodium hydroxide solution, for washing. The result was a print of photographic accuracy, with appearance as in the original, but with all gelatin removed, the silver having been moved radially outwardly and been deposited and held on the paper.

*Example 2*

A conventional photographic transparency and a conventional solution of Gelatinase No. 3 were used. The transparency and a sheet of blotting paper were placed, with the gelatin layer of the transparency radially outwardly and contacting thereover the blotting paper, against the perforated cylindrical ten-inch diameter bas-

ket 14 of the centrifuge shown in FIG. 1, which was rotated about the axis of the cylindrical surface of basket 14 to impose a centrifugal force of 15,000 times gravity, while there was simultaneously introduced warm Gelatinase No. 3 solution through pipe 16 for ten minutes. The centrifuge was then stopped and the film with which the gelatin has been integral was removed. The blotting paper, now bearing the silver particles, was then centrifuged for five more minutes while passing through further solution to dissolve any remaining bits of gelatin, and five more minutes with wash water, at all times at 15,000 times gravity. A print of photographic accuracy on the blotting paper resulted, silver particles appearing well below the surface thereof in relative densities preserving the image of the original transparency.

*Example 3*

The procedure set forth in Example 2 was repeated, except that glass cloth was used instead of blotting paper for a base. A gelatin-free print of photographic accuracy on glass cloth was obtained, which remained sharp and clear even after heating for one hour at 500° F.

*Example 4*

The gelatin layer of an ordinary photographic transparency, carrying silver particles defining a photographic image and constituting together therewith a developed and fixed photographic emulsion, was softened with a solution of Gelatinase No. 3. The surface of the softened gelatin layer was placed against the roughened surface of Mylar film roughened by "vapor-blasting" with finely divided grit to a finely frosted appearance, the other surface of the Mylar film being placed against a cylindrical imperforate centrifuge basket. As in the other examples above set forth, all portions of the gelatin or organic layer surface were equidistant from the axis of rotation of the basket, as were all portions of the support surface of the basket, as were all portions of the support surface in contact with the gelatin surface. The basket was then rotated for ten minutes in the presence of the solvent solution, to produce a force of 5,000 times gravity throughout the gelatin layer and against the roughened surface of the Mylar support. A print on Mylar, of photographic accuracy, resulted.

*Example 5*

A photographic print with a  $\frac{3}{16}'' \times \frac{5}{8}''$  image was placed on the flat bottom of a bottle, which was mounted on an arm parallel to the centerline of the bottle and perpendicular to its bottom. Softening, destruction of

4

the gelatin layer and washing were under the conditions set forth for Example 1, using a batch approach as there. Rotation was on said arm, the flat bottom of the bottle being  $10\frac{1}{2}$  inches from the axis of rotation and generally perpendicular to the radius extending from said axis through the center of said bottom. A print of photographic accuracy, free from gelatin, resulted.

Other embodiments within the invention and appended claim will occur to those skilled in the art, the embodiments of the above examples being exemplary only. My new process may desirably be used in making up labels, for example, with such high definition that they may be read only by means of a magnifying glass and with great heat resistance, or in the making up of prints of photographic accuracy on cloth, blotters, solid objects such as ashtrays, or other materials, which may be chosen for such characteristics as to flexibility, durability, heat resistance, porosity, and so on, as seem desirable for the end use required. Coatings, heat-resistant (such as of silicones) or otherwise, may be used on the receiving surface of the base, either before or after depositing thereon the solid particles defining thereon an image, to increase adhesion, protect against dirt or abrasion, or give a modified appearance.

I claim:

The method of manufacturing a print which comprises the steps of supporting against the cylindrical wall of a centrifuge basket a base and supporting against the base and inwardly thereof a layer of hydrophilic colloid carrying dispersed therein silver particles defining a photographic image, rotating said basket to give said base and said layer the same angular velocity, dissolving said hydrophilic colloid to release said silver particles therefrom, and moving said silver particles radially onto said base for retention thereon to give an image reproducing with photographic accuracy the image already referred to.

**References Cited by the Examiner**

**UNITED STATES PATENTS**

|           |         |                |       |           |
|-----------|---------|----------------|-------|-----------|
| 2,119,309 | 5/1938  | Batchelor      | ----- | 117—101 X |
| 2,339,131 | 1/1944  | Anderson       | ----- | 117—63 X  |
| 2,339,178 | 1/1944  | Lemmers        | ----- | 117—63 X  |
| 3,097,112 | 7/1963  | Schutze et al. | ----- | 117—101 X |
| 3,212,929 | 10/1965 | Pliskin et al. | ----- | 117—101 X |

ALFRED L. LEAVITT, Primary Examiner.

RALPH S. KENDALL, Examiner.